

# United States Patent [19]

Hanlon

[11] Patent Number: 4,482,356

[45] Date of Patent: Nov. 13, 1984

[54] **DIESEL FUEL CONTAINING ALKENYL SUCCINIMIDE**

[75] Inventor: J. Vincent Hanlon, Baton Rouge, La.

[73] Assignee: Ethyl Corporation, Richmond, Va.

[21] Appl. No.: 567,089

[22] Filed: Dec. 30, 1983

[51] Int. Cl.<sup>3</sup> .. C10L 1/22

[52] U.S. Cl. .. 44/57; 44/71;  
44/72

[58] Field of Search .. 44/57, 71, 72

[56] **References Cited**

**U.S. PATENT DOCUMENTS**

2,280,217 4/1942 Cloud .. 44/57  
3,490,882 1/1970 Dunworth .. 44/72  
3,909,215 9/1975 Kray .. 44/62

4,240,803 12/1980 Andress, Jr. .... 44/71

*Primary Examiner—Y. Harris-Smith*

*Attorney, Agent, or Firm—Donald L. Johnson; John F. Sieberth; Willard G. Montgomery*

[57]

## ABSTRACT

Coking in and around the injector nozzles of indirect injection compression ignition engines is reduced by means of distillate fuel with which has been blended suitable concentrations of:

- (a) organic nitrate ignition accelerator, and
- (b) hydrocarbyl-substituted succinimide.

Also described are additive mixtures of (a) and (b) for use in distillate fuels in amounts sufficient to reduce the coking tendencies of such fuels when used in the operation of indirect injection compression ignition engines.

49 Claims, 1 Drawing Figure





**DIESEL FUEL CONTAINING ALKENYL  
SUCCINIMIDE**

**FIELD**

Compression ignition fuel compositions and additive mixtures of organic nitrate ignition accelerator and hydrocarbyl-substituted succinimide, in amounts sufficient to resist the coking tendencies of compression ignition fuel compositions when used in the operation of indirect injection diesel engines.

**BACKGROUND**

Throttling diesel nozzles have recently come into widespread use in indirect injection automotive and light-duty diesel truck engines, i.e., compression ignition engines in which the fuel is injected into and ignited in a prechamber or swirl chamber. In this way, the flame front proceeds from the prechamber into the larger compression chamber where the combustion is completed. Engines designed in this manner allow for quieter and smoother operation.

The FIGURE of the drawing illustrates the geometry of the typical throttling diesel nozzle (often referred to as the "pintle nozzle").

Unfortunately, the advent of such engines has given rise to a new problem, that of excessive coking on the critical surfaces of the injectors that inject fuel into the prechamber or swirl chamber of the engine. In particular and with reference to the FIGURE, the carbon tends to fill in all of the available corners and surfaces of the obturator 10 and the form 12 until a smooth profile is achieved. The carbon also tends to block the drilled orifice 14 in the injector body 16 and fill up to the seat 18. In severe cases, carbon builds up on the form 12 and the obturator 10 to such an extent that it interferes with the spray pattern of the fuel issuing from around the perimeter of orifice 14. Such carbon build up or coking often results in such undesirable consequences as delayed fuel injection, increased rate of fuel injection, increased rate of combustion chamber pressure rise, and increased engine noise, and can also result in an excessive increase in emission from the engine of unburned hydrocarbons.

While low fuel cetane number is believed to be a major contributing factor to the coking problem, it is not the only relevant factor. Thermal and oxidative stability (lacquering tendencies), fuel aromaticity, and such fuel characteristics as viscosity, surface tension and relative density have also been indicated to play a role in the coking problem.

An important contribution to the art would be a fuel composition which has enhanced resistance to coking tendencies when employed in the operation of indirect injection diesel engines.

**THE INVENTION**

In accordance with one of its embodiments, this invention provides distillate fuel for indirect injection compression ignition engines containing at least the combination of (a) organic nitrate ignition accelerator, and (b) hydrocarbyl-substituted succinimide, said combination being present in an amount sufficient to minimize coking, especially throttling nozzle coking, in the prechambers or swirl chambers of indirect injection compression ignition engines operated on such fuel.

Another embodiment of the present invention is a distillate fuel additive fluid composition comprising (a)

organic nitrate ignition accelerator, and (b) hydrocarbyl-substituted succinimide in an amount sufficient to minimize the coking characteristics of such fuel, especially throttling nozzle coking, in the prechambers or swirl chambers of indirect compression ignition engines operated on such fuel.

Since the invention also embodies the operation of an indirect injection compression ignition engine in a manner which results in reduced coking, a still further embodiment of the present invention is a method of inhibiting coking, especially throttling nozzle coking, in the prechambers or swirl chambers of an indirect injection compression ignition engine, which comprises supplying said engine with a distillate fuel containing at least the combination of (a) organic nitrate ignition accelerator, and (b) hydrocarbyl-substituted succinimide, said combination being present in an amount sufficient to minimize such coking in an engine operated on such fuel.

A feature of this invention is that the combination of additives utilized in its practice is capable of suppressing coking tendencies of fuels used to operate indirect injection compression ignition engines. Such behavior was exhibited in a series of standard engine dynamometer tests conducted as described in Example I hereinafter.

A wide variety of organic nitrate ignition accelerators may be employed in the fuels of this invention. Preferred nitrate esters are the aliphatic or cycloaliphatic nitrates in which the aliphatic or cycloaliphatic group is saturated, contains up to about 12 carbons and, optionally, may be substituted with one or more oxygen atoms.

Typical organic nitrates that may be used are methyl nitrate, ethyl nitrate, propyl nitrate, isopropyl nitrate, allyl nitrate, butyl nitrate, isobutyl nitrate, sec-butyl nitrate, tert-butyl nitrate, amyl nitrate, isoamyl nitrate, 2-amyl nitrate, 3-amyl nitrate, hexyl nitrate, heptyl nitrate, 2-heptyl nitrate, octyl nitrate, isoctyl nitrate, 2-ethylhexyl nitrate, nonyl nitrate, decyl nitrate, undecyl nitrate, dodecyl nitrate, cyclopentyl nitrate, cyclohexyl nitrate, methylcyclohexyl nitrate, cyclododecyl nitrate, 2-ethoxyethyl nitrate, 2-(2-ethoxyethoxy)ethyl nitrate, tetrahydrofuranyl nitrate, and the like. Mixtures of such materials may also be used. The preferred ignition accelerator for use in the fuels of this invention is a mixture of octyl nitrates available as an article of commerce from Ethyl Corporation under the designation DII-3 ignition improver.

The hydrocarbyl-substituted succinimides, component (b) of the fuels of this invention, are well known. They are readily made by first reacting an olefinically unsaturated hydrocarbon of the desired molecular weight with maleic anhydride to form a hydrocarbyl-substituted succinic anhydride. Reaction temperatures of about 100°-250° C. are used. With higher boiling olefinically-unsaturated hydrocarbons, good results are obtained at about 200°-250° C. This reaction can be promoted by the addition of chlorine. Typical olefins include cracked wax olefins, linear alpha olefins, branched chain alpha olefins, polymers and copolymers of lower olefins. These include polymers of ethylene, propylene, isobutylene, 1-hexene, 1-decene and the like. Useful copolymers are ethylene-propylene copolymers, ethylene-isobutylene copolymers, propylene-isobutylene copolymers, ethylene-1-decene copolymers and the like.

Hydrocarbyl substituents have also been made from olefin terpolymers. Very useful products have been made from ethylene-C<sub>3</sub>-12 alpha olefin-C<sub>5</sub>-12 non-conjugated diene terpolymers; such as ethylene-propylene-1,4-hexadiene terpolymer; ethylenepropylene-1,5-cyclooctadiene terpolymer; ethylene-propylenenorbornene terpolymers and the like.

Of the foregoing, by far the most useful hydrocarbyl substituents are derived from butene polymers, especially polymers of isobutylene.

The molecular weight of the hydrocarbyl substituent can vary over a wide range. It is desirable that the hydrocarbyl group have a molecular weight of at least 500. Although there is no critical upper limit, a preferred range is about 500-500,000 number average molecular weight. The more preferred average molecular weight is about 700-5,000 and most preferably about 900-3,000.

Hydrocarbyl-substituted succinimides and succinamides are made by reaction of the desired hydrocarbyl-substituted succinic anhydride with an amine having at least one reactive hydrogen atom bonded to an amine nitrogen atom. Examples of these are methyl amine, dimethyl amine, n-butyl amine, di-(n-dodecyl) amine, N-(aminoethyl) piperidine, piperazine, N-(3-aminopropyl) piperazine, and the like.

Preferably, the amine has at least one reactive primary amine group capable of reacting to form the preferred succinimides. Examples of such primary amines are n-octyl amine, N,N-dimethyl-1,3-propane diamine, N-(3-aminopropyl) piperazine, 1,6-hexane diamine, and the like.

Hydroxylalkyl amines can also be used to make the succinimide-succinamide components of the invention which contain some ester groups. These amines include ethanol amine, diethanol amine, 2-hydroxypropyl amine, N-hydroxyethyl ethylenediamine and the like. Such hydroxylalkyl amines can be made by reacting a lower alkylene oxide, such as ethylene oxide, propylene oxide or butylene oxide with ammonia or a primary or secondary amine such as ethylene diamine, diethylene triamine, triethylene tetramine, tetraethylenepentamine and the like.

A more preferred class of primary amines used to make the succinimide, succinamide or mixtures thereof are the polyalkylene amines. These are polyamines and mixtures of polyamines which have the general formula



wherein R is a divalent aliphatic hydrocarbon group having 2-4 carbon atoms and n is an integer from 1-10 including mixtures of such polyalkylene amines.

In a highly preferred embodiment, the polyalkylene amine is a polyethylenamine containing about 2-6 ethylenamine units. These are represented by the above formula in which R is the group —CH<sub>2</sub>CH<sub>2</sub>— and n has a value of 2-6.

The amine used to make the succinimide, succinamide or mixture thereof need not be all amine. A mono or poly-hydroxyalcohol may be included in the reaction. Such alcohols can be reacted concurrently with the amine or the two alcohol and amine may be reacted sequentially. Useful alcohols are methanol, ethanol, n-dodecanol, 2-ethyl hexanol, ethylene glycol, propylene glycol, diethylene glycol, 2-ethoxy ethanol, trimethylol propane, pentaerythritol, dipentaerythritol and the like.

Useful amine-alcohol products are described in U.S. Pat. Nos. 3,184,474; 3,576,743; 3,632,511; 3,804,763; 3,836,471; 3,936,480; 3,948,800; 3,950,341; 3,957,854; 3,957,855; 3,991,098; 4,071,548 and 4,173,540.

The reaction between the hydrocarbyl-substituted succinic anhydride and the amine can be carried out by mixing the components and heating the mixture to a temperature high enough to cause a reaction to occur but not so high as to cause decomposition of the reactants or products or the anhydride may be heated to reaction temperature and the amine added over an extended period. A useful temperature is about 100°-250° C. Best results are obtained by conducting the reaction at a temperature high enough to distill out water formed in the reaction.

A preferred succinimide-succinamide component is available as an article of commerce from the Edwin Cooper Company under the designation HITEC ®E-644. This product comprises a mixture of active ingredients and solvent. Thus, when HITEC ®E-644 is used as component (b) in formulating the fuels of this invention, the product as received should be used at a concentration of at least about 40 PTB (pounds per thousand barrels) to insure that the finished blend contains an adequate quantity of the foregoing succinimide-succinamide ingredient although smaller amounts may be successfully employed.

The nitrate ignition accelerator—component (a)—should be present in an amount of at least 100 to 1000 PTB (pounds per thousand barrels) of the base fuel. Preferably, the concentration of the ignition accelerator is about 400 to 600 PTB.

It is not believed that there is anything critical as regards the maximum amount of components (a) and (b) used in the fuel. Thus, the maximum amount of these components will probably be governed in any given situation by matters of choice and economics.

The coking-inhibiting components (a) and (b) of the invention can be added to the fuels by any means known in the art for incorporating small quantities of additives into distillate fuels. Components (a) and (b) can be added separately or they can be combined and added together. It is convenient to utilize additive fluid mixtures which consist of organic nitrate ignition accelerator and hydrocarbyl-substituted succinimide-succinamide agents. These additive fluid mixtures are added to distillate fuels. In other words, part of the present invention are coking inhibiting fluids which comprise organic nitrate ignition accelerator and hydrocarbyl-substituted succinimide-succinamide.

Use of such fluids in addition to resulting in great convenience in storage, handling, transportation, blending with fuels, and so forth, also are potent concentrates which serve the function of inhibiting or minimizing the coking characteristics of compression ignition distillate fuels used to operate indirect compression ignition engines.

In these fluid compositions, the amount of components (a) and (b) can vary widely. In general, the fluid compositions contain about 5 to 95% by weight of the organic nitrate ignition accelerator component and 5 to 95% by weight of the hydrocarbyl-substituted succinimide-succinamide component. Typically, from about 0.01% by weight up to about 1.0% by weight of the combination will be sufficient to provide good coking-inhibiting properties to the distillate fuel. A preferred distillate fuel composition contains from about 0.1 to about 0.5% by weight of the combination containing

from about 25% to about 95% by weight of the organic nitrate ignition accelerator and from about 75% to about 5% by weight of the hydrocarbyl-substituted succinimide-succinamide component.

The additive fluids, as well as the distillate fuel compositions of the present invention may also contain other additives such as, corrosion inhibitors, antioxidants, metal deactivators, detergents, cold flow improvers, inert solvents or diluents, and the like.

Accordingly, a more preferred distillate fuel composition includes a hydrocarbyl amine in combination with the present additives.

While a variety of hydrocarbyl amines may be used in the fuel compositions of this invention, a primary aliphatic amine, the aliphatic group of which is tertiary, e.g., an amine of the formula:



wherein R is one or a mixture of tertiary aliphatic groups containing 8 to 18 or more (preferably 12-16) carbon atoms is preferred. Most preferably, these tertiary aliphatic groups are tertiary alkyl groups. It is also preferred that hydrocarbyl amine component (c) include in addition to the above-described amine one or more hydrocarbyl amines differing therefrom.

U.S. Pat. No. 3,909,215, all disclosure of which is incorporated herein, gives a description of the various hydrocarbyl amines having from 3 to 60 carbons and from 1 to 10 nitrogens which may be employed in the fuels of this invention. A few additional examples of desirable amines include 2,6-di-tert-butyl- $\alpha$ -dimethylamino-p-cresol, N-cyclohexyl-N,N-dimethylamine, and N-alkyl,N,N-dimethylamines in which the alkyl group is one or a combination of alkyl groups preferably having 8 to 18 or more carbon atoms.

A particularly preferred hydrocarbyl amine is available commercially from the Rohm and Haas Company under the designation Primene 81R. The Primene 81R is believed to be a mixture of primary aliphatic amines in which the aliphatic groups are predominantly C<sub>12</sub> and C<sub>14</sub> tertiary alkyl groups.

The fuels of this invention should contain at least 1.5 to 40 PTB of component (c), the hydrocarbyl amine.

Accordingly, another embodiment of the present invention is distillate fuel for indirect injection compression ignition engines containing at least the combination of (a) organic nitrate ignition accelerator, (b) hydrocarbyl-substituted succinimide, and (c) hydrocarbyl amine, said combination being present in an amount sufficient to minimize coking, especially throttling nozzle coking in the prechambers or swirl chambers in indirect injection compression ignition engines operated on such fuel.

Also included as a further embodiment of the invention is a distillate fuel additive composition comprising (a) organic nitrate ignition accelerator, (b) hydrocarbyl-substituted succinimide and (c) hydrocarbyl amine in an amount sufficient to minimize the coking characteristics of such fuel, especially throttling nozzle coking in the prechambers or swirl chambers in indirect injection compression ignition engines operated on such fuel.

In general, these additive fuel compositions will contain as much as 50% by weight of the combination of organic nitrate ignition accelerator and hydrocarbyl-substituted succinimide and up to 50% of the hydrocarbyl amine or other additives when they are present.

In a still further embodiment of the invention there is provided a method of inhibiting coking, especially throttling nozzle coking in the prechambers or swirl

chambers of an indirect injection compression ignition engine which comprises supplying said engine with a distillate fuel containing at least the combination of (a) organic nitrate ignition accelerator, (b) hydrocarbyl-substituted succinimide and (c) hydrocarbyl amine, said combination being present in an amount sufficient to minimize such coking in an engine operated on such fuel.

Another additive which can be used to advantage in the present invention is a metal deactivator. Examples of these are salicylidene-o-aminophenol, disalicylidene ethylenediamine and disalicylidene propylenediamine. A particularly preferred metal deactivator is N,N'-disalicylidene-1,2-diaminopropane (80 weight percent active in 20 weight percent toluene solvent) which is available as an article of commerce from Ethyl Corporation under the designation "Ethyl" MDA.

The fuels of this invention should contain at least 0.2 to 5 PTB of component (d), the metal deactivator, preferably N,N'-disalicylidene-1,2-diaminopropane.

Accordingly, another embodiment of the present invention is distillate fuel for indirect injection compression ignition engines containing at least the combination of (a) organic nitrate ignition accelerator, (b) hydrocarbyl-substituted succinimide, (c) hydrocarbyl amine, and (d) N,N'-disalicylidene-1,2-diaminopropane, said combination being present in an amount sufficient to minimize coking, especially throttling nozzle coking in the prechambers or swirl chambers in indirect injection compression ignition engines operated on such fuel.

Also included as a further embodiment of the invention is a distillate fuel additive composition comprising (a) organic nitrate ignition accelerator, (b) hydrocarbyl-substituted succinimide, (c) hydrocarbyl amine, and (d) N,N'-disalicylidene-1,2-diaminopropane in an amount sufficient to minimize the coking characteristics of such fuel, especially throttling nozzle coking in the prechambers or swirl chambers of indirect injection compression ignition engines operated on such fuels.

In general, these additive fuel compositions will contain as much as 50% by weight of the combination of organic nitrate ignition accelerator and hydrocarbyl-substituted succinimide-succinamide and up to 50% of the combination of hydrocarbyl amine and N,N'-disalicylidene-1,2-diaminopropane or other additives when they are present.

In a still further embodiment of the invention there is provided a method of inhibiting coking, especially throttling nozzle coking in the prechambers or swirl chambers in an indirect injection compression ignition engine which comprises supplying said engine with a distillate fuel containing at least the combination of (a) organic nitrate ignition accelerator, (b) hydrocarbyl-substituted succinimide, (c) hydrocarbyl amine and (d) N,N'-disalicylidene-1,2-diaminopropane, said combination being present in an amount to minimize such coking in an engine operated on such fuel.

The practice and advantages of this invention will become still further apparent from the following illustrative example.

#### EXAMPLE 1

In order to determine the effect of the fuel compositions of the present invention on the coking tendency of diesel injectors in indirect injection compression ignition engines, use was made of a commercial diesel engine operated on a coking test cycle developed by Insti-

tute Francais Petrole and as practiced by Peugeot S. A. The amount of coking together with a quantitative indication of the adverse consequences of such coking was determined by means of (i) injector air flow performance, (ii) emission of unburned hydrocarbons, (iii) engine noise, and (iv) injector deposit ratings. The engine employed in the tests was a 1982 Peugeot 2.3 liter, 4-cylinder, turbocharged XD2S diesel engine connected to a Midwest dynamometer through an engine clutch. This engine is equipped with Bosch injectors positioned within prechambers, and is deemed representative of the indirect injection compression ignition engines widely used in automobiles and light-duty trucks.

The base fuel employed in these engine tests was a commercially-available diesel fuel having a nominal cetane rating of 42. FIA analysis indicated the fuel was composed by volume of 31.5% aromatics, 3.0% olefins and 65.5% saturates. Its distillation range (ASTM D-158) was as follows:

|                |                    |  |
|----------------|--------------------|--|
| Barometer      | 29.46 inches of Hg |  |
| Initial        | 406° F.            |  |
| % Evaporated   | at °F.             |  |
| 5              | 439                |  |
| 10             | 450                |  |
| 15             | 456                |  |
| 20             | 463                |  |
| 30             | 480                |  |
| 40             | 499                |  |
| 50             | 521                |  |
| 60             | 545                |  |
| 70             | 572                |  |
| 80             | 603                |  |
| 85             | 621                |  |
| 90             | 643                |  |
| 95             | 678                |  |
| Final Recovery | 678° F.            |  |
| Residue        | 97.5%              |  |
| Loss           | 2.5%               |  |
|                | None               |  |

Other inspection data on the base fuel were as follows:

|                                   |                          |  |
|-----------------------------------|--------------------------|--|
| Kinematic Viscosity, (ASTM D-445) | 3.50 Centistokes, 40° C. |  |
| Pour Point (ASTM D-97)            | -26° C.                  |  |
| Cloud Point (ASTM D-97)           | 33° C.                   |  |
| Flash Point (ASTM D-93)           | 91° C.                   |  |
| Steam Jet Gum                     | 2.4 mg/100 ml            |  |
| Aniline Point (ASTM D-611)        | 143.4° F.                |  |
| Total Sulfur                      | 0.41 wt. %               |  |
| Ramsbottom Carbon, % (ASTM D-524) | 0.1460 on 10% Residuum   |  |
| Gravity (ASTM D-287)              | 31.8 °API                |  |
| Specific Gravity @ 25° C.         | 0.86                     |  |
| Cetane rating                     | 41                       |  |

A test blend was prepared from this base fuel (Fuel A). Fuel A contained a combination of (i) 506 PTB of mixed octyl nitrates (a commercial product available from Ethyl Corporation under the designation DII-3 Ignition Improver), (ii) 41 PTB of HITEC®E-644, a product of Edwin Cooper, Inc., believed to be a hydrocarbyl succinimide-succinamide made by reacting two moles of a polyisobutylene succinic anhydride (PIBSA) with one mole of a polyethylene amine mixture having an average composition corresponding to tetraethylene pentamine, (iii) 14 PTB of a hydrocarbyl amine available commercially from Rohm and Haas Company under the designation Primene 81R and (iv) 1.7 PTB of "Ethyl" Metal Deactivator, a product of Ethyl Corporation, the active ingredient of which is N,N'-disalicyli-

dene-1,2-diaminopropane. The manufacturer gives the following typical properties for its HITEC®E-644 product:

|                                  |                           |
|----------------------------------|---------------------------|
| Appearance                       | Dark brown viscous liquid |
| Nitrogen, wt. %                  | 2.0                       |
| Specific Gravity<br>at 60/60° F. | 0.928                     |
| Viscosity at 210° F., cs         | 340                       |

The Primene 81R is believed to be a mixture of primary aliphatic amines in which the aliphatic groups are predominantly C<sub>12</sub> and C<sub>14</sub> tertiary alkyl groups.

The manufacturer gives the following typical properties for its "Ethyl" metal Deactivator:

|                                 |                                        |
|---------------------------------|----------------------------------------|
| Form                            | Liquid                                 |
| Color                           | Amber                                  |
| Density, at 68° F.              |                                        |
| g/ml                            | 1.0672                                 |
| lb/gal                          | 8.91                                   |
| Active ingredient, wt %         | 80                                     |
| Solvent vehicle (toluene), wt % | 20                                     |
| Flash point, open cup, °F.      | 84                                     |
| Fire point, °F.                 | 100                                    |
| Solubility                      |                                        |
| In gasoline (Typical)           | Saturated solution<br>contains 94% MDA |
| In water, wt. %                 | 0.04                                   |

Shell Rotella T, an SAE 30, SF/CD oil was used as the crankcase lubricant.

Before starting each test, new Bosch DNOSD-1510 nozzles were installed using new copper gaskets and flame rings. The fuel line was flushed with the new test fuel composition to be tested and the fuel filter bowl and fuel return reservoir were emptied to avoid additive carry-over from test-to-test.

At the start of each test, the engine was operated at 1000 rpm, light load for 15 minutes. After this warm-up, the engine was subjected to the following automatic cycle:

| Event | RPM  | Beam Load | Minutes | EGR |
|-------|------|-----------|---------|-----|
| 1     | 750  | 0         | 4       | off |
| 2     | 2750 | 12.0      | 6       | on  |
| 3     | 1500 | 6.2       | 6       | on  |
| 4     | 4000 | 16.2      | 4       | off |

The above 20-minute cycle was repeated 60 times and the test was completed by running the engine at idle for another 30 minutes. The total elapsed time was thus 20.5 hours per test.

When passing from one event to the next event in the above cycle, some time, of course, was required to enable the engine to accelerate or decelerate from one speed to the next. Thus, more specifically, the above cycle was programmed as follows:

| Segment | Seconds | rpm  | Beam Load |
|---------|---------|------|-----------|
| 1       | 2       | 750  | 0         |
| 2       | 200     | 750  | 0         |
| 3       | 3*      | 2500 | 12        |
| 4       | 7*      | 2750 | 12        |
| 5       | 350     | 2750 | 12        |
| 6       | 3*      | 2275 | 6.2       |
| 7       | 7*      | 1500 | 6.2       |
| 8       | 330     | 1500 | 6.2       |

-continued

| Segment | Seconds | rpm  | Beam Load |
|---------|---------|------|-----------|
| 9       | 3*      | 3500 | 16.2      |
| 10      | 7*      | 4000 | 16.2      |
| 11      | 230     | 4000 | 16.2      |
| 12      | 3*      | 2000 | 0         |
| 13      | 7*      | 750  | 0         |
| 14      | 30      | 750  | 0         |

\*Represents two mode periods for acceleration or deceleration to the next condition.

Hydrocarbon exhaust emissions were measured at the start of each test (after the first 20-minute cycle), at the 6-hour test interval and at the end of the test. These measurements were made at 750, 1000, and 1400 rpm idle. Noise level readings were made at a location three feet from the engine exhaust side. The measurements were made at the start and at the end of the test while operating at three idle speeds, viz., 750, 1000 and 1400 rpm.

After the test operation, the injectors were carefully removed from the engine so as not to disturb the deposits formed thereon. Measurements were made of air flow through each nozzle at different pintle lifts, and pintle deposits were rated using the CRC deposit rating system.

The most significant test results are given in Table I, in which air flow is expressed as cc/min and hydrocarbon emissions as ppm.

TABLE I

| Fuel | Pintle Lift | Air Flow @ 0.1 mm |      | Obturator Deposits |      | Noise, DB |      | Hydrocarbon Emissions |  |
|------|-------------|-------------------|------|--------------------|------|-----------|------|-----------------------|--|
|      |             | (10 = clean)      | EOT* | INCR.              | EOT* | INCR.     | EOT* | INCR.                 |  |
| Base | 36          | 8.0               | 83.8 | 3.0                | 577  | 406       |      |                       |  |
| A    | 38          | 8.6               | 81.4 | 1.9                | 275  | 143       |      |                       |  |

\*Value at end of test; the increase (Incr.) shown is in comparison to the value at start of test.

The results presented in Table I show that there were less coking deposits (higher air flow rate and fewer deposits), less engine noise and less hydrocarbon emissions with Fuel A, the fuel of the invention, as compared to the Base Fuel.

I claim:

1. Distillate fuel for indirect injection compression ignition engines containing at least the combination of (a) organic nitrate ignition accelerator and (b) hydrocarbyl-substituted succinimide or succinamide, said combination being present in an amount sufficient to minimize coking in the nozzles of indirect injection compression ignition engines operated on such fuel.

2. The composition of claim 1 wherein said ignition accelerator is a mixture of octyl nitrates.

3. The composition of claim 1 wherein said hydrocarbyl-substituted succinimide is an olefin polymer substituted succinimide wherein said olefin polymer substituent has an average molecular weight of about 500-500,000.

4. The composition of claim 3 wherein the succinimide portion is derived from a polyalkyleneamine having the formula



wherein R is a divalent aliphatic hydrocarbon group having 2-4 carbon atoms and n is an integer from 1-10 including mixtures of said polyalkylene amines.

5. The composition of claim 4 wherein said olefin polymer substituent is a polyisobutene substituent.

6. The composition of claim 5 wherein said polyisobutene substituent has an average molecular weight of about 700-5,000.

7. The composition of claim 6 wherein said polyalkylene amine is a polyethyleneamine.

8. The composition of claim 7 wherein said polyethylene amine contains about 2-6 ethylene amine units.

9. A method of inhibiting coking on the injector nozzles of indirect injection compression ignition engines, 10 which method comprises supplying said engine with a distillate fuel containing at least the combination of (a) organic nitrate ignition accelerator and (b) hydrocarbyl-substituted succinimide or succinamide, said combination being present in an amount sufficient to minimize such coking in the engine operated on such fuel.

10. The method of claim 9 wherein said ignition accelerator is a mixture of octyl nitrates.

11. The method of claim 9 wherein said hydrocarbyl-substituted succinimide is an olefin polymer substituted succinimide wherein said olefin polymer substituent has an average molecular weight of about 500-500,000.

12. The process of claim 11 wherein the succinimide portion is derived from a polyalkylene amine having the formula



wherein R is a divalent aliphatic hydrocarbon group having 2-4 carbon atoms and n is an integer from 1-10 including mixtures of said polyalkylene amines.

13. The process of claim 12 wherein said olefin polymer substituent is a polyisobutene substituent.

14. The process of claim 13 wherein said polyisobutene substituent has an average molecular weight of about 700-5,000.

15. The process of claim 14 wherein said polyalkylene amine is a polyethylene amine.

16. The process of claim 15 wherein said polyethylene amine contains about 2-6 ethylene amine units.

17. Distillate fuel for indirect injection compression ignition engines containing at least the combination of (a) organic nitrate ignition accelerator, (b) hydrocarbyl-substituted succinimide or succinamide, (c) hydrocarbyl amine having from 3 to 60 carbons and from 1 to 10 nitrogens, said combination being present in an amount sufficient to minimize coking on the nozzles of indirect injection compression ignition engines operated on such fuel.

18. Distillate fuel for indirect injection compression ignition engines containing at least the combination of (a) organic nitrate ignition accelerator, (b) hydrocarbyl-substituted succinimide or succinamide, (c) hydrocarbyl amine having from 3 to 60 carbons and from 1 to 10 nitrogens, and (d) N,N'-disalicylidene-1,2-diaminopropane, said combination being present in an amount sufficient to minimize coking on the nozzles of indirect injection compression ignition engines operated on such fuel.

19. The composition of claim 17 wherein said ignition accelerator is a mixture of octyl nitrates.

20. The composition of claim 17 wherein said hydrocarbyl-substituted succinimide is an olefin polymer-substituted succinimide wherein said olefin polymer substituent has an average molecular weight of about 500-500,000.

21. The composition of claim 20 wherein the succinimide portion is derived from a polyalkyleneamine having the formula



wherein R is a divalent aliphatic hydrocarbon group having 2-4 carbon atoms and n is an integer from 1-10 including mixtures of said polyalkyleneamines.

22. The composition of claim 21 wherein said olefin polymer substituent is a polyisobutylene substituent.

23. The composition of claim 22 wherein said polyisobutylene substituent has an average molecular weight of about 700-5000.

24. The composition of claim 23 wherein said polyalkyleneamine is a polyethylene amine.

25. The composition of claim 24 wherein said polyethylene amine contains about 2-6 ethylene amine units.

26. The composition of claim 17 wherein said hydrocarbyl amine is comprised of an alkylene amine of the formula

20



wherein R is one or a mixture of tertiary alkyl groups containing 8 to 18 carbon atoms.

27. The composition of claim 26 wherein R is one or a mixture of tertiary alkyl groups containing 12-16 carbon atoms.

28. The composition of claim 18 wherein said ignition accelerator is a mixture of octyl nitrates.

29. The composition of claim 18 wherein said hydrocarbyl-substituted succinimide is an olefin polymer-substituted succinimide wherein said olefin polymer substituent has an average molecular weight of 500-500,000.

30. The composition of claim 29 wherein the succinimide portion is derived from a polyalkyleneamine having the formula



40

wherein R is a divalent aliphatic hydrocarbyl group having 2-4 carbon atoms and n is an integer from 1-10 including mixtures of said polyalkyleneamines.

31. The composition of claim 30 wherein said olefin polymer substituent is a polyisobutylene substituent.

32. The composition of claim 31 wherein said polyisobutylene substituent has an average molecular weight of about 700-500,000.

33. The composition of claim 32 wherein said polyalkyleneamine is a polyethylene amine.

34. The composition of claim 33 wherein said polyethylene amine contains about 2-6 ethylene amine units.

35. The composition of claim 18 wherein said hydrocarbyl amine is comprised of an alkylene amine of the formula



50

wherein R is one or a mixture of tertiary alkyl groups containing 8 to 18 carbon atoms.

36. The composition of claim 35 wherein R is one or a mixture of tertiary alkyl groups containing 12-16 carbon atoms.

37. An additive fluid concentrate for use in distillate fuels containing at least the combination of (a) organic nitrate ignition accelerator and (b) hydrocarbyl-substituted succinimide or succinamide.

38. A concentrate of claim 37 wherein said ignition accelerator is a mixture of octyl nitrates.

39. A concentrate of claim 37 wherein said hydrocarbyl-substituted succinimide is an olefin polymer substituted succinimide wherein said olefin polymer substituent has an average molecular weight of about 500-500,000.

40. A concentrate of claim 39 wherein the succinimide portion is derived from a polyalkyleneamine having the formula



wherein R is a divalent aliphatic hydrocarbon group having 2-4 carbon atoms and n is an integer from 1-10 including mixtures of said polyalkyleneamines.

41. A concentrate of claim 40 wherein said olefin polymer substituent is a polyisobutylene substituent.

42. A concentrate of claim 41 wherein said polyisobutylene substituent has an average molecular weight of about 700-5,000.

43. A concentrate of claim 42 wherein said polyalkyleneamine is a polyethylene amine.

44. A concentrate of claim 43 wherein said polyethylene amine contains about 2-6 ethylene amine units.

45. A concentrate of claim 37 comprising about 5-95% by weight of said organic nitrate ignition accelerator and about 5-95% of said hydrocarbyl substituted succinimide or succinamide.

46. An additive fluid concentrate for use in distillate fuels containing at least the combination of (a) organic nitrate ignition accelerator, (b) hydrocarbyl-substituted succinimide or succinamide and (c) hydrocarbyl amine having from 3 to 60 carbons and from 1 to 10 nitrogens.

47. A concentrate of claim 46 comprising up to about 50% by weight of the combination of organic nitrate ignition accelerator and hydrocarbyl-substituted succinimide or succinamide and up to about 50% by weight of said hydrocarbyl amine.

48. An additive fluid concentrate for use in distillate fuels containing at least the combination of (a) organic nitrate ignition accelerator, (b) hydrocarbyl-substituted succinimide or succinamide, (c) hydrocarbyl amine and (d) N,N'-disalicylidene-1,2-diaminopropane.

49. A concentrate of claim 48 comprising up to about 50% by weight of the combination of organic nitrate ignition accelerator and hydrocarbyl substituted succinimide or succinamide and up to about 50% by weight of the combination of said hydrocarbyl amine and N,N'-disalicylidene-1,2-diaminopropane.

\* \* \* \* \*

60

UNITED STATES PATENT AND TRADEMARK OFFICE  
CERTIFICATE OF CORRECTION

PATENT NO. : 4,482,356

DATED : November 13, 1984

INVENTOR(S) : J. Vincent Hanlon

It is certified that error appears in the above-identified patent and that said Letters Patent is hereby corrected as shown below:

Column 3, line 49, reads " $H_2N\{R-NH\}_nH$ " and should read  
--  $H_2N\{R-NH\}_nH$  --.

Column 5, line 51, reads "of swirl chambers" and should read -- or swirl chambers --.

Column 9, line 62, reads " $H_2N\{R-NH\}_nH$ " and should read  
--  $H_2N\{R-NH\}_nH$  --.

Column 10, line 26, reads " $H_2N\{R-NH\}_nH$ " and should read  
--  $H_2N\{R-NH\}_nH$  --.

Column 11, line 2, reads " $H_2N\{R-NH\}_nH$ " and should read  
--  $H_2N\{R-NH\}_nH$  --.

Column 11, line 40, reads " $H_2N\{R-NH\}_nH$ " and should read  
--  $H_2N\{R-NH\}_nH$  --.

Column 12, line 21, reads " $H_2N\{R-NH\}_nH$ " and should read  
--  $H_2N\{R-NH\}_nH$  --.

**Signed and Sealed this**

*Thirtieth Day of April 1985*

[SEAL]

*Attest:*

**DONALD J. QUIGG**

*Attesting Officer*

*Acting Commissioner of Patents and Trademarks*